

## 1

2,878,296

## CORROSION INHIBITED FLUIDS

Robert S. Montgomery, Midland, Mich., assignor to The Dow Chemical Company, Midland, Mich., a corporation of Delaware

No Drawing. Application December 5, 1956  
Serial No. 626,281

7 Claims. (Cl. 260—652.5)

This invention relates to and has for its principal objective the provision of certain media comprised of base fluids consisting of halogenated hydrocarbons that are not corrosive to various metal surfaces, particularly iron and steel surfaces, and which are especially utile for employment as hydraulic fluids, as coolants in metal heat-exchanging systems and for like purposes.

According to the present invention, a non-corroductive medium is comprised of a base fluid of the indicated type containing a minor proportion of a miscible alkyl ester of coal acids in which the alkyl radical contains less than about twenty and preferably from about seven to thirteen carbon atoms in its structure. Advantageously, the base fluid may be rendered non-corrosive to metals to provide a medium in accordance with the invention by incorporating therein between about 0.01 and 5 percent by weight of the alkyl ester of coal acids, based on the weight of the non-corroductive medium. For many purposes it may be more advantageous to employ from 0.1 to 2 percent by weight of the alkyl ester of coal acids in the medium.

It is desirable for the alkyl ester of coal acids that is employed to be a completely or substantially completely esterified product. Such an ester may be obtained readily as the product of the reaction of free coal acids with suitable alcohols and in other ways analogous to those in which ordinary polycarboxylic acids are conventionally esterified. As indicated, it is of particular benefit in some cases for at least about a seven carbon atom alkyl radical to be employed in the ester. Esters of this variety tend to be more readily miscible with a larger proportion of the base fluids that are contemplated as being within the scope of the invention. Typical of the esters which may advantageously be utilized in the practice of the invention are the isoctyl; 2-ethyl-n-hexyl; decyl; lauryl; tridecyl and oleyl esters of coal acids and the like as well as their mixtures.

As mentioned, the base fluids that may be rendered non-corrosive by the alkyl esters of coal acids consist of liquid halogenated hydrocarbons, including fluorinated, chlorinated, brominated and mixed-halogenated derivatives exclusive of iodine-containing compounds. Practice of the invention is exceptionally advantageous with certain chlorofluorocarbons such as hexachlorotetrafluorobutane ( $C_4Cl_6F_4$ ) and the like which are exceptionally useful as hydraulic fluids (as, for example, in the hydraulic operating systems for airplane landing gear) but

## 2

which tend to be extremely corrosive to most of the metals that are commonly employed in such systems.

The coal acids that are employed to prepare the esters utilized in the present invention may be identical with or similar to those which may be obtained in a known manner by the oxidation with gaseous oxygen of an aqueous alkaline slurry of a finely divided carbonaceous material selected from the group consisting of coal and coke that has been obtained by the carbonization of coal at temperatures beneath about 700° C. Coal acids that have been obtained by the nitric acid oxidation of suitable carbonaceous materials are also generally satisfactory.

The free coal acids are hygroscopic, usually yellowish, essentially water-soluble material. They are believed to be comprised substantially of various aromatic polycarboxylic acids in a mixture having an average molecular weight in the neighborhood of 250. Their average equivalent weight is generally about eighty. They ordinarily appear to have an average of two and one-half to five carboxylic groups per molecule with an apparent average of three to four being common. While their exact chemical nature and constitution may be somewhat conjectural, they evidently contain considerable quantities of tri-and tetra-carboxylic benzene acids as well as aromatic acids having more complex nuclei. Frequently, for example, the greatly preponderant proportion of aromatic nuclei obtained in the conventionally manufactured coal acids may be found to consist of methylnaphthalene, benzene, biphenyl, naphthalene, phenanthrene, alkyl benzene, benzophenone and toluene nuclei.

To afford additional delineation, several alkyl esters of coal acids were tested for their efficacy in inhibiting the corrosiveness upon metals of hexachlorotetrafluorobutane. In testing the halogenated hydrocarbon, about one percent by weight proportions of each of the alkyl esters of coal acids that were tested were incorporated in the base fluid. About seventy-five gram portions of each of the thus-inhibited base fluids were added to a sealable six-ounce glass container along with about twenty-five grams of distilled water. A one-quarter by two and one-half inch strip, having a thickness of about three-sixty-fourths of an inch, of Formula 52-100 cold rolled steel, wrapped crosswise with seven turns and lengthwise with one turn of No. 19 copper wire, was inserted in each of the containers. The containers were then tightly sealed and tumbled for about forty-eight hours at a temperature of about 200° F. At the termination of this period, the copper and steel specimens from each of the bottles were examined closely for evidences of corrosion and the steel strip checked for possible weight loss. Each of the corrosion-inhibited fluids were analyzed for possible changes in their viscosity and increases in acidity. The results which were obtained in each of the tests that was conducted are set forth in the following tabulation which also includes certain of the physical properties of the particular esters that were utilized for testing purposes.

| Corrosion-Inhibiting Ester of Coal Acids | Viscosity of Ester in centipoises at 100° F. | Viscosity of Ester in centipoises at 210° C. <sup>a</sup> | Viscosity Index of Ester <sup>a</sup> | Pour Point of Ester in °F. <sup>b</sup> | Specific Gravity of Ester at 25/25° C. | Corrosion-Inhibiting Properties In Test With $C_4Cl_6F_4$ |
|------------------------------------------|----------------------------------------------|-----------------------------------------------------------|---------------------------------------|-----------------------------------------|----------------------------------------|-----------------------------------------------------------|
| Isooctyl.....                            | 629                                          | 30.05                                                     | 76                                    | 0                                       | (e)                                    | Excellent.                                                |
| 2-Ethyl-n-hexyl.....                     | 695                                          | 32.45                                                     | 78                                    | -5                                      | (e)                                    | Do.                                                       |
| Decyl.....                               | 96                                           | 12.16                                                     | 120                                   | -20                                     | 0.963                                  | Do.                                                       |
| Lauryl.....                              | 195                                          | 20.23                                                     | 119                                   | +35                                     | 0.955                                  | Good.                                                     |
| Tridecyl.....                            | 900                                          | 37.23                                                     | 76                                    | +10                                     | 0.973                                  | Do.                                                       |
| Oleyl.....                               | 83.76                                        | 13.50                                                     | 140                                   | +25                                     | (e)                                    | Do.                                                       |

<sup>a</sup>As determined by A.S.T.M. D-445-53T for viscosity and D-567-53 for viscosity index.

<sup>b</sup>As determined by A.S.T.M. D-97-47.

<sup>c</sup>Not determined.

In comparison, tests conducted with uninhibited control samples caused extreme corrosion of the metal specimens from the halogenated hydrocarbon. None of the inhibited hexachlorotetrafluorobutane fluids that were tested showed any appreciable change in viscosity or acid number after the tests. Likewise, no appreciable weight loss was discernible in the metal specimens tested in the halogenated hydrocarbon fluids.

What is claimed is:

1. Non-corrodon composition comprised of a base fluid consisting of a normally liquid halogenated hydrocarbon in which there is dispersed a minor proportion that is not in excess of about 5 percent by weight, based on the weight of said composition, of a miscible alkyl ester of coal acids in which the alkyl radical contains less than about twenty carbon atoms in its structure; said coal acids being the water soluble mixed aromatic polycarboxylic acids that are the products of the oxidation of coal and the like carbonaceous materials, which acids typically have an average molecular weight of about 250, an average apparent equivalent weight of about 80, and contain an average of from about two and one-half to

five carboxylic groups per aromatic nuclei in their molecule.

2. The composition of claim 1 containing from about 0.1 to 2 percent by weight of the dispersed ester.

3. Non-corrodon composition comprised of a normally liquid chlorofluorocarbon fluid in which there is dispersed between about 0.01 and 5 percent by weight of an alkyl ester of coal acids in which the alkyl radical contains from about seven to thirteen carbon atoms.

4. The composition of claim 3, wherein the ester is the isoocetyl ester of coal acids.

5. The composition of claim 3, wherein the ester is the 2-ethyl-n-hexyl ester of coal acids.

6. The composition of claim 3, wherein the ester is the decyl ester of coal acids.

7. The composition of claim 3, wherein the chlorofluorocarbon fluid is hexachlorotetrafluorobutane.

#### References Cited in the file of this patent

#### UNITED STATES PATENTS

2,516,640 Montgomery et al. July 25, 1950